

1

2,988,514

**BLEACHING COMPOSITION AND METHOD**

Homer L. Robson, Lewiston, N.Y., Lorenzo D. Taylor, St. Petersburg, Fla., and Richard R. Heinze, Ransomville, N.Y., assignors to Olin Mathieson Chemical Corporation

No Drawing. Filed June 11, 1958, Ser. No. 741,216  
25 Claims. (Cl. 252—187)

This invention relates to improvements in bleaching 10 using acid solutions of a chlorite.

In the bleaching of cellulosic materials, including particularly pulp and textile, an acid solution of a chlorite is commonly used to obtain maximum bleaching and the production of goods of high whiteness. A typical bleach 15 bath used in textile work contains, for example, approximately one gram per liter of sodium chlorite. Sufficient acid is added to the bath with or without buffering to bring the pH to the desired value, generally to a pH of about 3.5 for cotton goods or about 2.5 for polyacrylonitrile fiber. Acetic acid is the preferred acid for achieving the pH of 3.5 and formic acid is the preferred acid for achieving the pH of 2.5. Phosphoric acid is also frequently used as an acidifying agent. Buffer salts, for example,  $\text{Na}_2\text{HPO}_4$ ,  $\text{NaH}_2\text{PO}_4$  or  $\text{NH}_4\text{HF}_2$  can be added. In addition, wetting agents which are effective under acid conditions, for example, the "Igepions" (salts of acylalkyl taurides) are commonly added. Bleaching baths of these compositions are commonly used at elevated temperatures, for example 180° F. to 195° F.

Under these conditions of use, the bleaching solutions generate chlorine dioxide rather rapidly, as evidenced by the development of a yellow color in the solution and by the evolution of chlorine dioxide as a gas from the surface of the solution. This generation of chlorine dioxide is objectionable in that the gas lost from the solution represents a loss in bleaching power. It is also objectionable as a health hazard when sufficient chlorine dioxide is evolved to affect workers deleteriously. Chlorine dioxide is an irritating gas and requires removal, for example, by means of hoods from the working space. Furthermore, acid chlorite solutions, particularly when chlorine dioxide is being evolved in the range of pH 2 to pH 4, are corrosive to stainless steels and other metals. These metals become pitted and then corrode at a faster rate than the original highly polished surfaces. In addition, the corrosion products in the solution frequently stain the textile and accelerate further decomposition of the chlorite to chlorine dioxide. Thus, it is necessary, for the most economical and efficient bleaching, to acidify the bleaching bath to form chlorous acid and/or chlorine dioxide at a rate matching the demand on the solution by the textile being bleached and, at the same time, to avoid producing an excess of chlorine dioxide which would saturate the solution and be evolved as a gas.

Fine adjustment of the pH of the bleaching bath is difficult and, by itself, is inadequate to provide sufficient chlorine dioxide, as opposed to too much chlorine dioxide. Control of the rate of formation of chlorine dioxide has been attempted by starting the bleach at a moderate temperature, such as 160° F. and a moderate pH of about 4 and adding acid and increasing the temperature during the bleaching period to activate the remaining chlorite more strongly. But such procedures require constant manual attention and it is more desirable, in any event, to add sufficient acid at the beginning for the entire process and to maintain constant temperature.

Considerable control of the corrosion aspect of the excessive chlorine dioxide production problem can be effected by addition to the bleaching bath of nitric acid as the acidifying agent or the addition to the bleaching bath of inorganic nitrates up to a molar ratio of 0.5/1

2

or more of nitrate to chlorite. For some fabrics, such as "Dacron" (a polyethylene terephthalate fiber), the use of nitric acid or nitrates has been specified by the manufacturer when chlorite bleaching is employed. Many textile plants, however, regard nitric acid as dangerous to handle. Moreover, control of pH using nitric acid is difficult, since it has no buffering action. Consequently, some mills have preferred to add nitrate salts, e.g., sodium nitrate, to the bath along with the other ingredients and to employ acetic acid as the acidifying agent. Acetic acid has a pronounced and useful buffering action, tending to hold the pH value somewhat constant or, at least, minimizing its rise as the bleach bath is used. The addition of sodium nitrate or other nitrate salts to the bath does not interfere with the buffering action. However, there is a limit to the ability of nitrates to retard corrosion of stainless steel in acidified chlorite solutions; to reduce the amounts of corrosion products, particularly iron compounds which cause the decomposition of the chlorite and the production of chlorine dioxide; and to overcome the adverse effects of, for example, iron which may be introduced into the bleach bath from other sources.

Thus, it is seen that there are needed means and methods which repress excessive evolution of chlorine dioxide in baths containing all the necessary acid at the beginning of the bleaching operation. One such method of repressing the formation of chlorine dioxide with hydrogen peroxide is described in U.S. Patent No. 2,358,866, issued September 26, 1944, to J. D. MacMahon. U.S. Patent No. 2,526,839, issued October 24, 1950, to R. N. Aston, describes the use of pyrophosphates and polyphosphates alone or with hydrogen peroxide for the same purpose. However, hydrogen peroxide and the polyphosphates are effective in acid solutions having a pH of about 3 and inordinately large amounts of these repressers are required at lower pH levels. Consequently, what have been sought are more effective and more economical repressers in the pH 2 to pH 3 range to lessen decomposition of the chlorite and formation of chlorine dioxide. Such repressers would be assisted by the use of nitrates to reduce the amounts of corrosion products, particularly iron compounds, in the bleach baths.

A principal object of the present invention is to provide an acidic aqueous bleach bath in which the active bleaching agent is supplied in the form of a water-soluble chlorite and in which there are additionally contained novel repressers which are particularly effective in preventing the formation of chlorine dioxide in such amounts as will cause the evolution thereof from the bath as a gas and which act without interfering with the bleaching action of the bath.

Another object of the present invention is to provide a concentrated aqueous composition suitable for addition to an acidified aqueous bleach bath to produce a buffered solution which is substantially non-corrosive to stainless steel and which contains the novel repressers. The active bleaching agents in the bath are supplied in the form of water-soluble metal chlorites.

A third object of the present invention is to provide a concentrated, stable, solid composition suitable for addition to an acidified bleach bath to produce a buffered solution which is substantially non-corrosive to stainless steel and which contains the novel repressers. The active bleaching agents in the bath are supplied in the form of water-soluble metal chlorites.

The chlorite component of the bleaching bath is most commonly sodium chlorite which is commercially available, although any of the alkali metal or alkaline earth metal chlorites are suitable, for example, lithium chlorite, potassium chlorite or calcium chlorite. In most bleaching operations, a concentration of about 0.1 to 5 grams per

liter of sodium chlorite are used, but, in some circumstances up to 20 grams per liter or more can be used. Equivalent amounts of  $\text{LiClO}_2$ ,  $\text{KClO}_2$  or  $\text{Ca}(\text{ClO}_2)_2$  can also be used.

The novel repressers employed are polyamides of the general formula:



in which R is hydrogen or methyl and n is 1 to 4. Ethylene diamine is a particularly preferred repressor and is conveniently introduced into the bleaching bath as the dihydrochloride. Other amines within the scope of the formula are diethylene triamine, triethylene tetramine, tetraethylene pentamine, propylene diamine, dipropylene triamine, and other propylene homologues of these polyamines, and mixtures thereof. The hydrochlorides or phosphate salts of these amines are useful forms in which the amines may be obtained, handled and introduced into the bleaching bath.

Many amines repress the formation of chlorine dioxide from acidic chlorite solutions. However, they may form inactive chloroamines which have no bleaching action or they may be so reactive as to reduce the active bleaching agents in the solution and rob it of available oxidizing power. Again, other amines form colors which are objectionable in a bleaching process. By contrast, the polyamines of the formula



where R is H or methyl and n is 1 to 4 are very effective in repressing the formation of chlorine dioxide in the aqueous acidic chlorite solutions at pH values from the neutral point of 7 to as low as about 2 without these adverse effects. The proportions of polyamine required are suitably in the range of 10 to 1000 parts per million by weight in a bleaching bath containing about 1000 to 2000 parts by million by weight of sodium chlorite or equivalent amounts of other water-soluble chlorites. Observable effects begin at about 10 parts per million by weight of the polyamine and more than about 500 parts per million by weight appear to be of no additional advantage over somewhat smaller amounts. The proportion of repressor is related, as described, to the chlorite content of the bleaching bath and is varied with the chlorite content, so as to maintain the proportion set forth. And, in such proportion, these polyamines are surprisingly effective in repression, particularly when compared with other nitrogen-bearing compounds and with other proposed repressers, even in the presence of known accelerators of chlorine dioxide formation. Triethylene tetramine, for example, represses chlorine dioxide formation, even in the presence of 2 parts per million by weight of iron, though not as well as it does in the absence of iron.

Thus, when using the polyamines defined above in the presence of dissolved iron, there may be some loss of total effective bleaching power in the bath. Ordinarily, this is not excessive unless the proportion of iron is excessive and, if iron is absent, there is substantially no loss of bleaching power. If the polyamines combine in any way with the active bleaching agents, the products are also active bleaching agents. They reduce the formation of chloride or chlorate from the chlorite and thereby preserve the bleaching power of the chlorite. They do not form any colored by-products which might interfere with bleaching textiles to high whiteness. They are stable and effective repressers at operating temperatures between room temperature and the boiling point of the solution. They are compatible with other components of the bleaching baths.

In addition to the chlorite, the acid and the polyamines discussed above, the bleaching bath of the present invention advantageously contains conventional ingredients, such as buffers, corrosion inhibitors, wetting agents and metal ion chelating agents. Suitable buffers include, for example,  $\text{Na}_2\text{HPO}_4$ ,  $\text{NaH}_2\text{PO}_4$ ,  $\text{NH}_4\text{HF}_2$ , sodium acetate,

and acetic acid. These buffers tend to keep the pH of the solution constant in spite of the introduction of materials tending to neutralize the acid, raise the pH, and thereby reduce or stop the bleaching action.

- 5 In bleaching textiles with acidified chlorite solutions, wetting agents stable and effective in such solutions are commonly added to the bleaching bath. When sodium chlorite was introduced to the textile trade, a study was made of the various wetting agents which might be used. 10 Members of the "Igepon" (salts of acylalkyl taurides) series were found to be the most satisfactory of those tested. The "Igepon T" compounds (salts of higher acyl derivatives of lower alkyltaurides), particularly the oleoyl derivatives, are especially useful. Baths containing these 15 wetting agents have somewhat longer life than those made with other wetting agents. Accordingly, "Igepon T" wetting agents were generally recommended to the textile trade for use with acidic chlorite solutions and many textile mills continue to employ them.
- 20 Equipment employed in bleaching textiles with chlorite is commonly made of stainless steel. The stainless steel may be combined with sheets of glass, Transite (a hard pressed, heavy board or tubing made from asbestos and Portland cement), and other inert materials. Particularly 25 with intermittent use for chlorite baths, stainless steel may show some corrosion, sufficient to add one part per million by weight of iron to the bleach bath or a sufficient fraction of a part per million to affect the course of the bleaching adversely, e.g., by accelerating chlorine dioxide 30 formation and evolution, by acting antagonistically toward the repressers, by introducing discoloration, and by damaging the equipment being employed. Nickel and cobalt which may be dissolved from the stainless steel act similarly to the iron in these regards. Again, these 35 metals may appear in the bleaching bath due to corrosion or they may be otherwise, often inadvertently, introduced. Whatever their source, they are deleterious and their introduction is to be avoided if possible. Indeed, it is preferred in the practice of this invention to take positive 40 steps to remove such metals if they have been introduced.

To reduce the corrosion of stainless steel and to prevent the introduction of deleterious metal ions therefrom into the bleaching bath, a water-soluble nitrate salt is preferably included in the bath. Ammonium nitrate and alkali metal and alkaline earth metal nitrates such as sodium nitrate, potassium nitrate, calcium nitrate or magnesium nitrate are preferably employed. A suitable proportion of up to about 0.50 mole of nitrate per mole of chlorite is used. Such proportions materially reduce corrosion and introduction of deleterious metal ions from stainless steel into the bleaching solution.

To inactivate traces of the deleterious metal ions which have been introduced, the bleaching solution can contain, 55 in a preferred modification of the present invention, a chelating agent which is stable with respect to the bleaching components and effective in acid solution. A study of the effect of iron on the repressing action of various amines showed that iron either weakened the repressing 60 action or was itself so strong a catalyst in the formation of chlorine dioxide that, to obtain optimum repression, inactivation of the iron is required. In glass equipment with iron completely absent, some repressers give good repression of the chlorine dioxide, resulting in long bath life and more even bleaching of the goods being treated. 65 The same test made in metal equipment shows poor repression, due to a small pick-up of iron.

The chelating agents useful in the present invention are those amines having a plurality of hydrogen atoms of the amino group replaced by fatty carboxylic acid groups. 70 Particularly useful members of this group include ethylene diamine tetra-acetic acid, hydroxyethyl-ethylene diamine triacetic acid, iminodiacetic acid, nitrilo-triacetic acid, symmetrical ethylene-diamine diacetic acid and their 75 salts, generally alkali metal salts, such as sodium salts.

Also useful are citric, maleic, lactic and tartaric acid and salts of citric acid and tartaric acid, for example, alkali metal salts such as sodium citrate and sodium potassium tartrate. These chelating agents are effective at the pH used in acidified chlorite bleaching baths to minimize the action of iron and other metal ions, such as nickel and cobalt, in engendering the formation of chlorine dioxide. Ordinarily, about 5 to 50 parts per million by weight, based on the solution are satisfactory.

Thus, to summarize what has been said concerning the bleaching bath solutions of the present invention, these aqueous compositions include from about 0.1 and 20 grams per liter of sodium chlorite or equivalent weights of other water-soluble chlorites, are given a pH within the range of 2 to 7, and contain at least one polyamine of the formula



in an amount sufficient to prevent the evolution of chlorine dioxide gas from the bath but insufficient in amount to destroy the bleaching potential of the chlorite. R in the formula is selected from the group consisting of H and methyl and n is an integer from 1 to 4. For all practical purposes, this means that the polyamines are present in proportions of about 10 to 1000 parts per million by weight in baths containing about 1000 to 2000 parts per million by weight of sodium chlorite or equivalent amounts of other chlorites. These solutions can also contain an alkali metal or an alkaline earth metal nitrate in an amount of up to 0.50 mole of nitrate per mole of chlorite to serve as a corrosion inhibitor and suitable amounts of buffering agents, wetting agents and chelating agents.

The aqueous concentrates within the ambit of the present invention differ from the bleaching baths discussed above in that they contain neither water-soluble chlorite nor acid. They contain an alkali metal or alkaline earth metal nitrate such as sodium nitrate, potassium nitrate, lithium nitrate or calcium nitrate and they contain a polyamine of the type previously discussed. Advantageously, they also contain a chelating agent. The proportion of each component in the mixture is adjusted to provide a composition which, when introduced into an acidified chlorite solution, provides a bleaching bath which is substantially non-corrosive to stainless steel, suitably repressed with respect to chlorine dioxide formation and still effective under normal bleaching operation conditions. To this end, the following composition is generally suitable:

| Component:      | Percent by weight |
|-----------------|-------------------|
| Nitrate         | 20-32             |
| Polyamine       | 5-15              |
| Chelating agent | 3-10              |
| Water           | Balance           |
|                 | 100               |

Where particularly low temperatures may be encountered, it is preferable to use about 30 percent by weight of the nitrate component to lower the freezing point. Where the nitrate is an alkaline earth metal nitrate, it is preferable to use about 8 to 10 percent by weight of the chelating agent to obtain clear concentrates.

The non-aqueous components of the concentrates of the invention are all readily soluble in water in the recited proportions to form clear, stable solutions of a pH of about 11 to 12. The concentrates themselves freeze only below 0° F. and are easily prepared, stored, and shipped. When diluted by addition to an acidified chlorite solution, these concentrates yield a bleaching bath which is effective, stable, substantially non-corrosive and does not generate obnoxious quantities of chlorine dioxide. Suitable proportions are about 0.5 to 1.3 grams of the concentrate per gram of a commercial bleaching product containing from 80 to 84 percent by weight of

sodium chlorite or an equivalent amount of another water-soluble chlorite used in bleaching baths. Smaller proportions may protect only inadequately and greater amounts slow the bleaching process, although they do not impair the bleaching capacity of the bath. The concentrated aqueous compositions of the present invention are completely soluble in water and are effective repressers, especially at a pH of 2 to 3, without destroying bleaching power.

The solid compositions within the scope of the present invention differ from the bleaching baths discussed above in that they contain neither water-soluble chlorite, acid nor water. They contain an alkali metal nitrate such as sodium nitrate, potassium nitrate or lithium nitrate, but generally, they do not contain alkaline earth metal nitrates because of their hygroscopic nature. They contain a polyamine of the above noted formula, preferably in the form of a hydrochloride or phosphate salt. They also contain a buffering agent. Disodium phosphate is the preferred buffer, but sodium dihydrogen phosphate, polyphosphates, e.g., tetrasodiumpyrophosphate and sodium tripolyphosphate, as well as ammonium bifluoride and sodium acetate, can be employed. These buffers tend to hold the pH constant when chlorine dioxide is formed according to the equation:



since they replace the acid in the solution. Advantageously, these compositions also contain chelating agents of the type discussed above. The proportion of each component in the mixture is adjusted to provide a composition which, when introduced into an acidified chlorite solution, provides a bleach bath which is non-corrosive to stainless steel, suitably repressed with respect to chlorine dioxide formation and still effective in bleaching under normal operating conditions. To this end, the following composition is generally suitable:

| Component:          | Percent by weight |
|---------------------|-------------------|
| Nitrate             | 30 to 55          |
| Buffer              | 25 to 50          |
| Polyamine (or salt) | 4 to 12           |
| Chelating agent     | 3 to 20           |
|                     | 100               |

These components are preferably finely ground and admixed in any suitable manner, as by ball-milling or tumbling, to form a homogeneous mixture. The solid composition of the present invention is readily soluble in water and is an effective repressor, particularly at a pH of 2 to 3, without being destructive of bleaching power.

Within the following limits, the solid compositions, when dissolved in suitable proportions in an acidified chlorite solution, yield a bleaching bath which is effective, stable, substantially non-corrosive and does not generate obnoxious quantities of chlorine dioxide. Suitable proportions are about 0.5 to 1.0 gram of the solid per gram of a commercial bleaching product containing 80 percent by weight sodium chlorite used in the bleaching bath. Smaller proportions may protect only inadequately and greater amounts slow the bleaching process, although they do not impair the bleaching capacity of the bath. Larger proportions of nitrate in the composition are accommodated by decreasing the proportion of buffer. When the nitrate is in the 45 to 55 weight percent range, the proportion is reduced to about 0.5 gram per gram of sodium chlorite product, maintaining the molar ratio of nitrate to chlorite below about 0.50/1 in the bleach bath.

For a further understanding of the present invention, reference is made to the following examples:

#### Examples I-VIII

A solution containing 860 parts per million by weight

of sodium chlorite was buffered at pH 3.0 by the addition of 30 grams per liter of glacial acetic acid and 0.5 gram per liter of sodium acetate. It was divided into several portions to each of which was added a different proportion of a polyamine product having the following composition:

| Compound:                      | Weight, percent |
|--------------------------------|-----------------|
| Ethylenediamine and water      | 1.0             |
| Diethylenetriamine             | 80.0            |
| Triethylenetetramine           | 12.0            |
| Higher polyethylene polyamines | 7.0             |
|                                | 100.0           |

Each solution was maintained at 88° C. for various periods, removing a portion of the solution from time to time and chilling to stop further generation of chlorine dioxide. The content of dissolved chlorine dioxide in each sample in parts per million by weight was determined photometrically. When the concentration of free, dissolved chlorine dioxide had reached a fairly constant value, the run was stopped. The ability of the polyamines to reduce materially the formation of chlorine dioxide and thus to prolong the life of the bath is clearly shown in the following table:

8

of acetic acid-sodium acetate buffer. To one portion of the solution was added 500 parts per million by weight of triethylene tetramine. To another portion, 500 parts per million by weight of triethylene tetramine and 2 parts per million by weight of ferric chloride were added. A third portion was used as a blank. The solutions were maintained at 88° C., removing samples from time to time and determining the parts per million by weight of chlorine dioxide. After 30 minutes, the total content of sodium chlorite and dissolved chlorine dioxide was determined with the following results:

| Time, Min. | ClO <sub>2</sub> , p.p.m. |           | ClO <sub>2</sub> and NaClO <sub>2</sub> , p.p.m. |           |
|------------|---------------------------|-----------|--------------------------------------------------|-----------|
|            | No Re-presser             |           | With Re-presser                                  |           |
|            | No Iron                   | With Iron | No Iron                                          | With Iron |
| 0          | 0                         | 0         | 860                                              | 860       |
| 5          | 130                       | 0         | 22                                               |           |
| 10         | 160                       | 0         | 16                                               |           |
| 20         | 160                       | 0         | 8                                                |           |
| 30         | 160                       | 0         | 8                                                | 620       |
|            |                           |           | 860                                              | 210       |

| Example No.                       |  | I   | II  | III | IV  | V   | VI  | VII | VIII |
|-----------------------------------|--|-----|-----|-----|-----|-----|-----|-----|------|
|                                   |  | 0   | 20  | 50  | 100 | 160 | 200 | 300 | 400  |
| Chlorine Dioxide Produced, p.p.m. |  |     |     |     |     |     |     |     |      |
| Polyamine, p.p.m.                 |  |     |     |     |     |     |     |     |      |
| Time in Minutes:                  |  | 100 | 45  | 22  | 20  | 18  | 18  | 16  | 10   |
| 1                                 |  | 110 | 60  | 25  | 22  | 18  | 18  | 16  | 10   |
| 2                                 |  | 120 | 70  | 30  | 25  | 18  | 18  | 16  | 10   |
| 3                                 |  | 120 | 80  | 35  | 30  | 18  | 18  | 16  | 10   |
| 4                                 |  | 130 | 100 | 40  | 35  | 18  | 18  | 16  | 10   |
| 5                                 |  | 140 | 110 | 45  | 40  | 22  | 18  | 16  | 10   |
| 7                                 |  | 160 | 130 | 55  | 45  | 25  | 18  | 16  | 10   |
| 9                                 |  | 160 | 140 | 70  | 55  | 30  | 18  | 16  | 10   |
| 12                                |  | 160 | 150 | 90  | 65  | 40  | 22  | 18  | 10   |
| 15                                |  | 160 | 120 | 90  | 50  | 30  | 22  | 14  | 6    |
| 20                                |  | 160 | 130 | 120 | 70  | 40  | 30  | 16  | 8    |
| 25                                |  | 160 | 130 | 130 | 80  | 50  | 40  | 20  | 10   |
| 30                                |  | 160 | 130 | 130 | 90  | 50  | 50  | 30  | 12   |
| 40                                |  |     |     |     |     | 60  | 50  | 30  | 16   |
| 50                                |  |     |     |     |     | 50  |     |     |      |
| 60                                |  |     |     |     |     | 50  |     |     |      |

#### Example IX

A solution containing 860 parts per million by weight of sodium chlorite was buffered at pH 3 by adding an acetic acid-sodium acetate buffer. To one portion of the solution was added 500 parts per million by weight of ethylene diamine. Another portion was used as a blank. The solutions were maintained at 88° C., removing samples from time to time and determining the parts per million by weight of chlorine dioxide. After 30 minutes, the total content of sodium chlorite and dissolved chlorine dioxide was determined with the following results:

| Time, Min. | ClO <sub>2</sub> , p.p.m. |                 | ClO <sub>2</sub> and NaClO <sub>2</sub> , p.p.m. |                 |
|------------|---------------------------|-----------------|--------------------------------------------------|-----------------|
|            | No Re-presser             | With Re-presser | No Re-presser                                    | With Re-presser |
| 0          | 0                         | 0               | 860                                              | 860             |
| 5          | 130                       | 40              |                                                  |                 |
| 10         | 160                       | 65              |                                                  |                 |
| 20         | 160                       | 140             |                                                  |                 |
| 30         | 160                       | 160             | 620                                              | 760             |

These data show that the repressor slowed considerably the evolution of chlorine dioxide, at the same time preserving the bleaching power of the solution in the form of chlorine dioxide and chlorite.

#### Example X

A solution containing 860 parts per million by weight of sodium chlorite was buffered at pH 3 by the addition

50 of 500 parts per million by weight of triethylene tetramine. To another portion, 500 parts per million by weight of triethylene tetramine and 2 parts per million by weight of ferric chloride were added. A third portion was used as a blank. The solutions were maintained at 88° C., removing samples from time to time and determining the parts per million by weight of chlorine dioxide. After 30 minutes, the total content of sodium chlorite and dissolved chlorine dioxide was determined with the following results:

55

#### Example XI

60 A bleaching bath was made up containing 0.925 gram per liter of a commercial bleaching product containing 80 weight per cent NaClO<sub>2</sub>, equivalent to 1200 parts per million by weight of available chlorine. Eight milliliters of 56 weight percent aqueous acetic acid and 0.5 gram of caustic soda were added per liter to adjust the pH to 3. Then 0.5 gram per liter of "Igepon T-77" (sodium salt of oleoyl methyl tauride) wetting agent was dissolved 65 in the solution. To one portion of this solution were added 10 parts per million by weight of diethylenetriamine trihydrochloride and to another portion none was added. The solutions were heated to 86° C. for one hour in the presence of a sample of polyethylene terephthalate fiber-cotton textile using 15 grams per 500 milliliters of bleach solution (solution to cloth ratio by weight, 33/1). The cloth originally had a brightness of 58, measured using a Photovolt brightness meter. Chlorine dioxide content of the solution was determined on samples 70 removed at intervals. At the end of one hour, the cloths 75 removed at intervals. At the end of one hour, the cloths

were removed, rinsed, dried, ironed and the brightness determined. Results are shown in the following table:

| Experiment No.                              | 1    | 2    | 3    | 4    |
|---------------------------------------------|------|------|------|------|
| DETA.3HCl <sup>a</sup> added, p.p.m.        | 0    | 0    | 10   | 10   |
| Bath Analysis, (ClO <sub>2</sub> , p.p.m.): |      |      |      |      |
| Time, Min.—                                 |      |      |      |      |
| 15                                          | 48   | 88   | 25   | 20   |
| 30                                          | 70   | 70   | 48   | 38   |
| 60                                          | 100  | 110  | 88   | 76   |
| Brightness of Bleached Cloth                | 81.7 | 81.8 | 81.6 | 81.8 |

<sup>a</sup> Diethylene triamine trihydrochloride.

In each of the pairs of tests, agreement is satisfactory. The data clearly show the repressive influence of the DETA. No significant difference appears in the brightness of the bleached cloth.

#### Example XII

A bleaching bath was made up containing 0.925 gram per liter of a commercial bleaching product containing 80 weight percent NaClO<sub>2</sub>, equivalent to 1200 parts per million of available chlorine. Eight milliliters of 56 weight percent aqueous acetic acid and 0.5 gram of caustic soda were added per liter to adjust the pH to 3. Then 0.5 gram per liter of "Igepon T-77" wetting agent was dissolved in the solution. To separate portions of this solution were added various proportions of ethylenediamine dihydrochloride and to another portion none was added. The solutions were heated to 86° C. for one hour in the presence of a sample of polyethylene terephthalate fiber-cotton textile using 15 grams per 500 milliliters of bleach solution (solution to cloth ratio by weight, 33/1). The cloth originally had a brightness of 58, measured using a Photovolt brightness meter. Chlorine dioxide content of the solution was determined on samples removed at intervals. At the end of one hour, the cloths were removed, rinsed, dried, ironed and the brightness determined. Results are shown in the following table:

| Experiment No.                              | 1    | 2    | 3    | 4    | 5    | 6    | 7    |
|---------------------------------------------|------|------|------|------|------|------|------|
| EDA.2HCl <sup>a</sup> , p.p.m.              | 0    | 10   | 10   | 25   | 50   | 50   | 100  |
| Bath Analysis, (ClO <sub>2</sub> , p.p.m.): |      |      |      |      |      |      |      |
| Time, Min.—                                 |      |      |      |      |      |      |      |
| 15                                          | 38   | 85   | 25   | 24   | 18   | 18   | 14   |
| 30                                          | 70   | 64   | 53   | 42   | 35   | 26   | 24   |
| 60                                          | 110  | 94   | 94   | 76   | 64   | 52   | 42   |
| Brightness of Bleached Cloth                | 81.8 | 79.8 | 79.7 | 80.6 | 81.4 | 81.4 | 81.7 |

<sup>a</sup> Ethylenediamine dihydrochloride.

Where duplicate tests were run, agreement is satisfactory. The data clearly show the repressive influence of the ethylenediamine dihydrochloride. In each case, the chlorine dioxide content of the solution was reduced by increasing amounts of the polyamine. No significant difference appears in the brightness of the bleached cloth.

#### Example XIII

This example shows the effectiveness of one of the polyamines in repressing chlorine dioxide formation in the presence of iron using ethylenediamine tetra-acetic acid as chelating agent.

A bleaching bath was made up containing 0.925 gram per liter of a commercial product containing 80 weight percent NaClO<sub>2</sub>, equivalent to 1200 parts per million of available chlorine. Eight milliliters of 56 percent aqueous acetic acid and 0.5 gram of caustic soda were added per liter to adjust the pH to 3. Then 0.5 gram per liter of "Igepon T-77" wetting agent was dissolved in the solution. To separate portions of this solution were added various proportions of ethylenediamine dihydrochloride, ferric chloride and ethylenediamine tetra-acetic acid with suitable blanks. The solutions were heated to 86° C. for one hour in the presence of a sample of a polyethylene

terephthalate fiber-cotton textile using 15 grams per 500 milliliters of bleach solution (solution to cloth ratio by weight, 33/1). The cloth originally had a brightness of 58, measured using a Photovolt brightness meter. Chlorine dioxide content of the solution was determined on samples removed at intervals. At the end of one hour, the cloths were removed, rinsed, dried, ironed and the brightness determined. Results are shown in the following table:

| Experiment No.                            | 1    | 2    | 3    | 4    | 5    | 6    |
|-------------------------------------------|------|------|------|------|------|------|
| Iron, <sup>a</sup> p.p.m.                 | 0    | 0    | 10   | 10   | 10   | 10   |
| EDA.2HCl <sup>b</sup> , p.p.m.            | 0    | 100  | 0    | 100  | 100  | 0    |
| Chelating Agent, <sup>c</sup> p.p.m.      | 0    | 0    | 0    | 0    | 100  | 100  |
| Bath Analysis, ClO <sub>2</sub> , p.p.m.: |      |      |      |      |      |      |
| Time, Minutes—                            |      |      |      |      |      |      |
| 15                                        | 48   | 20   | 76   | 64   | 16   | 48   |
| 30                                        | 70   | 34   | 100  | 88   | 24   | 70   |
| 60                                        | 100  | 64   | 100  | 88   | 48   | 76   |
| Brightness of Bleached cloth              | 81.7 | 80.9 | 79.8 | 79.9 | 80.7 | 81.6 |

<sup>a</sup> Ferric chloride added.

<sup>b</sup> Ethylenediamine dihydrochloride.

<sup>c</sup> Ethylenediamine tetra-acetic acid sodium salt.

These data show the chlorine dioxide formation in No. 1 in the absence of iron, polyamine or chelating agent. No. 2 shows repression of chlorine dioxide in No. 1 by addition of ethylenediamine dihydrochloride. No. 3 shows the accelerating effect on chlorine dioxide formation by the addition of iron. No. 4 shows the repression by the polyamine, even in the presence of iron. No. 5 shows the special benefit of polyamine and chelating agent together in repressing chlorine dioxide formation. No. 6 shows that the chelating agent alone is not wholly responsible for this improved result, but both the polyamine and chelating agent are necessary.

#### Example XIV

This example shows the additional use of sodium nitrate in the bleach baths of the present invention.

A bleaching bath was made up containing 0.925 gram per liter of a commercial product containing 80 weight percent NaClO<sub>2</sub>. The pH was brought to 3 by the addition of acetic acid and 0.5 gram per liter of "Igepon T-77" wetting agent was added. Two portions of this solution were used as blanks. To each of two other portions were added 100 parts per million by weight of ethylenediamine dihydrochloride, 50 p.p.m. by weight of "Versene" (ethylene diamine tetra-acetic acid sodium salt) and 360 p.p.m. by weight of sodium nitrate. Swatches of a polyethylene terephthalate fiber-cotton cloth weighing 15 grams were introduced into each solution, including the blanks and they were then stirred at 85° C. for one hour. The swatches were removed and the brightness determined for comparison with the original brightness of 60.0. The following data were obtained:

| Experiment No.                  | 1    | 2    | 3    | 4    |
|---------------------------------|------|------|------|------|
| EDA.2HCl <sup>a</sup> , p.p.m.  | 0    | 0    | 100  | 100  |
| "Versene" <sup>b</sup> , p.p.m. | 0    | 0    | 50   | 50   |
| NaNO <sub>3</sub> , p.p.m.      | 0    | 0    | 360  | 360  |
| ClO <sub>2</sub> , p.p.m.       | 210  | 202  | 127  | 131  |
| Brightness of cloth             | 79.8 | 78.9 | 70.4 | 80.0 |

<sup>a</sup> Ethylenediamine dihydrochloride.

<sup>b</sup> Ethylenediamine tetra-acetic acid sodium salt.

#### Example XV

One liter of water containing 30 grams of acetic acid and 0.5 gram of sodium hydroxide, together with 0.5 gram of propylenediamine (500 parts per million by weight), was maintained at 88° C. One gram of 86 weight percent sodium chlorite was added and the chlorine dioxide content of the solution was determined at intervals spectrophotometrically. A blank was run with-

out the propylenediamine and the following results were obtained:

| Time in Minutes | Chlorine Dioxide, p.p.m. |                |
|-----------------|--------------------------|----------------|
|                 | No Repressor             | With Repressor |
| 0               | 0                        | 0              |
| 5               | 130                      | 20             |
| 10              | 160                      |                |
| 15              | 160                      | 30             |
| 30              |                          | 40             |

*Example XVI*

A solution containing 860 parts per million by weight of sodium chlorite was buffered at pH 3 by adding an acetic acid-sodium acetate buffer. A portion of this solution was used as a blank. To the remainder of the solution was added 500 parts per million by weight of ethylene diamine. A portion of this solution was used in test No. 1. To the remainder of the solution was added 2 parts per million by weight of ferric chloride. A portion of this solution was used in test No. 2. To the remainder of the solution was added 400 parts per million by weight of citric acid. This solution was used in test No. 3. Each of the test solutions was maintained at 88° C. for 30 minutes, removing samples from time to time and determining the parts per million by weight of chlorine dioxide. The total content of chlorine dioxide and dissolved sodium chlorite was determined in the final sample. The following results were obtained:

| Test No.    | ClO <sub>2</sub> , p.p.m. |     |     |    | ClO <sub>2</sub> and NaClO <sub>2</sub> , p.p.m. |     |     |     |
|-------------|---------------------------|-----|-----|----|--------------------------------------------------|-----|-----|-----|
|             | Blank                     | 1   | 2   | 3  | Blank                                            | 1   | 2   | 3   |
| Time, Min.: |                           |     |     |    |                                                  |     |     |     |
| 0           | 0                         | 0   | 0   | 0  | 860                                              | 860 | 860 | 860 |
| 5           | 130                       | 40  | 110 | 12 |                                                  |     |     |     |
| 10          | 160                       | 65  | 160 | 12 |                                                  |     |     |     |
| 20          | 180                       | 140 | 190 | 16 |                                                  |     |     |     |
| 30          | 160                       | 160 | 400 | 22 | 620                                              | 760 | 180 | 800 |

These data show that the repressor, in the absence of iron (test No. 1), slowed considerably the evolution of chlorine dioxide, at the same time preserving the bleaching power of the solution in the form of chlorine dioxide and chlorite. The iron, even in the presence of the repressor, materially accelerated the evolution of chlorine dioxide (to 400 p.p.m. by weight after 30 minutes) and destroyed much of the bleaching power of the solution (180 p.p.m. by weight combined chlorine dioxide and chlorite remaining after 30 minutes). Further addition of citric acid as chelating agent in test No. 3 overcame the effect of the added iron and even improved the action of the repressor (only 22 p.p.m. by weight of dissolved chlorine dioxide after 30 minutes). The citric acid also preserved the bleaching power of the solution (800 parts per million by weight of chlorine dioxide and chlorite remained after 30 minutes).

*Example XVII*

A solution containing 860 parts per million by weight of sodium chlorite was buffered at pH 3 by adding an acetic acid-sodium acetate buffer. A portion of this solution was used as a blank. To the remainder of the solution was added 500 parts per million by weight of triethylene tetramine. A portion of this solution was used in test No. 1. To the remainder of the solution was added 2 parts per million by weight of ferric chloride. A portion of this solution was used in test No. 2. To the remainder of the solution was added 400 parts per million by weight of citric acid. This solution was used in test No. 3. Each of the test solutions was maintained

at 88° C. for 30 minutes, removing samples from time to time and determining the parts per million by weight of chlorine dioxide. The total content of chlorine dioxide and dissolved sodium chlorite was determined in the final sample. The following results were obtained:

| Test No. |             | ClO <sub>2</sub> , p.p.m. |    |    |   | Blank | 1   | 2   | 3   |
|----------|-------------|---------------------------|----|----|---|-------|-----|-----|-----|
|          |             | Blank                     | 1  | 2  | 3 |       |     |     |     |
| 10       | Time, Min.: |                           |    |    |   |       |     |     |     |
| 0        | 0           | 0                         | 0  | 0  | 0 | 860   | 860 | 860 | 860 |
| 5        | 130         | 0                         | 22 | 8  |   |       |     |     |     |
| 10       | 160         | 0                         | 16 | 8  |   |       |     |     |     |
| 20       | 160         | 0                         | 8  | 14 |   |       |     |     |     |
| 30       | 160         | 0                         | 8  | 8  | 8 | 620   | 860 | 210 | 790 |

These data show that the repressor, in the absence of iron (test No. 1) substantially stopped the evolution of chlorine dioxide, at the same time preserving the bleaching power of the solution in the form of chlorine dioxide and chlorite. The iron, even in the presence of the repressor (test No. 2), accelerated the evolution of chlorine dioxide (to 22 p.p.m. by weight after 5 minutes) and destroyed much of the bleaching power of the solution (210 p.p.m. by weight combined chlorine dioxide and chlorite remaining after 30 minutes). Further addition of citric acid as chelating agent in test No. 3 controlled the effect of the added iron and preserved the bleaching power of the solution (790 parts per million by weight of chlorine dioxide and chlorite remained after 30 minutes).

*Example XVIII*

A solution containing 860 parts per million by weight of sodium chlorite was buffered at pH 3 by adding an acetic acid-sodium acetate buffer. A portion of this solution was used as a blank. To the remainder of the solution was added 500 parts per million by weight of triethylene tetramine. A portion of this solution was used in test No. 1. To the remainder of the solution was added 2 parts per million by weight of ferric chloride. A part of this solution was used in test No. 2. To the remainder of the solution was added 400 parts per million by weight of tartaric acid. This solution was used in test No. 3. Each of the test solutions was maintained at 88° C. for 30 minutes, removing samples from time to time and determining the parts per million by weight of chlorine dioxide. The total content of chlorine dioxide and dissolved sodium chlorite was determined in the final sample. The following results were obtained:

| Test No. |             | ClO <sub>2</sub> , p.p.m. |    |    |   | ClO <sub>2</sub> and NaClO <sub>2</sub> , p.p.m. |     |     |     |
|----------|-------------|---------------------------|----|----|---|--------------------------------------------------|-----|-----|-----|
|          |             | Blank                     | 1  | 2  | 3 | Blank                                            | 1   | 2   | 3   |
| 50       | Time, Min.: |                           |    |    |   |                                                  |     |     |     |
| 0        | 0           | 0                         | 0  | 0  | 0 | 860                                              | 860 | 860 | 860 |
| 5        | 130         | 0                         | 22 | 16 |   |                                                  |     |     |     |
| 10       | 160         | 0                         | 16 | 16 |   |                                                  |     |     |     |
| 20       | 160         | 0                         | 8  | 16 |   |                                                  |     |     |     |
| 30       | 160         | 0                         | 8  | 16 |   | 620                                              | 860 | 210 | 380 |

These data show that the repressor, in the absence of iron (test No. 1) substantially stopped the evolution of chlorine dioxide, at the same time preserving the bleaching power of the solution in the form of chlorine dioxide and chlorite. The iron, even in the presence of the repressor (test No. 2), accelerated the evolution of chlorine dioxide (to 22 p.p.m. by weight after 5 minutes) and destroyed much of the bleaching power of the solution (210 p.p.m. by weight combined chlorine dioxide and chlorite remaining after 30 minutes). Further addition of tartaric acid as chelating agent in test No. 3 controlled the effect of the added iron and improved retention of the bleaching power of the solution (380 parts per million by weight of chlorine dioxide and chlorite remained after 30 minutes).

13

## Example XIX

An aqueous concentrate of the following composition was prepared:

| Component                                          | Percent by weight |
|----------------------------------------------------|-------------------|
| Sodium nitrate.....                                | 30                |
| Ethylenediamine.....                               | 10                |
| Ethylenediamine tetra-acetic acid sodium salt..... | 5                 |
| Water.....                                         | 55                |
| Total.....                                         | 100               |

A bleach bath was prepared by dissolving 0.9 gram per liter of this solution and 1.0 gram per liter of a commercial product containing 80 weight percent  $\text{NaClO}_2$  in water. The addition of 20 milliliters of 56 percent acetic acid per liter of solution brought the pH to 3.0. A swatch of a polyethylene terephthalate fiber-cotton was introduced into a solution having a solution/cloth weight ratio of 30/1 and the mixture was stirred at  $85^\circ\text{C}$ . for one hour with a stainless steel stirrer. The chlorine dioxide content of the solution was determined photometrically from time to time and at the end of one hour the swatch was removed, rinsed, dried, ironed and the brightness determined using a Photovolt brightness meter with a "tristimulus" green filter (original brightness, 60.0). A blank was run omitting the aqueous concentrate of the present invention and the following comparative results were obtained:

| Chlorine dioxide, p.p.m. | Blank | With additive |
|--------------------------|-------|---------------|
| 0 minutes.....           | 0     | 0             |
| 15 minutes.....          | 95    | 15            |
| 30 minutes.....          | 120   | 40            |
| 60 minutes.....          | 165   | 70            |
| Brightness of Cloth..... | 80    | 80            |

The data show that chlorine dioxide was maintained at all times at a materially lower level in the bath with additive but the same bleaching effect was obtained in the same time.

## Example XX

An aqueous concentrate was prepared by dissolving the following components in water in the proportions indicated:

| Component                                           | Percent by Weight |
|-----------------------------------------------------|-------------------|
| Sodium nitrate.....                                 | 30                |
| Ethylene diamine.....                               | 10                |
| Ethylene diamine tetra-acetic acid sodium salt..... | 5                 |
| Water.....                                          | 55                |
| Total.....                                          | 100               |

A bleach bath was prepared by dissolving 1.0 gram per liter of a commercial product containing 80 weight percent  $\text{NaClO}_2$  in water, adding ferric chloride to provide 5 parts per million by weight of iron. To separate portions of this solution were added varying amounts of the concentrate described above reserving one portion as a blank. Each portion was adjusted to pH 3.0 by the addition of acetic acid and a swatch of a polyacrylonitrile fiber cloth was introduced into the solution (which has a solution to cloth weight ratio of 30/1). Original brightness, determined using a Photovolt brightness meter and a "tristimulus" green filter was 83. The solutions were stirred using a type 316 stainless steel stirrer at  $85^\circ\text{C}$ . for 1 hour, determining the chlorine dioxide content of the solution at intervals. At the end of one hour the cloths were removed, rinsed, dried, ironed and the brightness again measured. The following results were obtained:

| Test No.                  | 1    | 2    | 3    | 4    |
|---------------------------|------|------|------|------|
| Concentrate added:        |      |      |      |      |
| ml./l.....                | 0    | 0.5  | 0.75 | 1.0  |
| g./l.....                 | 0    | 0.6  | 0.9  | 1.2  |
| Final pH.....             | 4.2  | 3.0  | 3.0  | 3.2  |
| Chlorine dioxide, p.p.m.: |      |      |      |      |
| 0 minutes.....            | 0    | 0    | 0    | 0    |
| 15 minutes.....           | 100  | 35   | 25   | 21   |
| 30 minutes.....           | 100  | 65   | 50   | 45   |
| 60 minutes.....           | 90   | 95   | 90   | 90   |
| Brightness.....           | 84.1 | 88.0 | 86.2 | 86.2 |

## Example XXI

A concentrate of the following composition was prepared by dissolving the following components in water in the proportions indicated:

| Component                                          | Percent by Weight |
|----------------------------------------------------|-------------------|
| Sodium nitrate.....                                | 30                |
| Ethylenediamine.....                               | 10                |
| Ethylenediamine tetra-acetic acid sodium salt..... | 5                 |
| Water.....                                         | 55                |
| Total.....                                         | 100               |

A bleach bath was prepared by dissolving 1.0 gram per liter of a commercial product containing 80 weight percent  $\text{NaClO}_2$  in water, adding ferric chloride to provide 5 parts per million by weight of iron. To separate portions of this solution were added varying amounts of the concentrate described above reserving one portion as a blank. Each portion was adjusted to a pH of 2.5 by the addition of a mixture of 2 volumes of concentrated nitric acid to 1 volume of glacial acetic acid and swatches of a polyacrylonitrile fiber cloth were introduced (solution to cloth weight ratio, 30/1). Original brightness, determined using a Photovolt brightness meter and a "tristimulus" green filter was 83. The solutions were stirred using a type 316 stainless steel stirrer at  $85^\circ\text{C}$ . for 1 hour, determining the chlorine dioxide content of the solution at intervals. At the end of one hour the cloths were removed, rinsed, dried, ironed and the brightness again measured. The following results were obtained:

| Test No.                  | 1    | 2    | 3    | 4    |
|---------------------------|------|------|------|------|
| Concentrate added:        |      |      |      |      |
| ml./l.....                | 1    | 0.5  | 0.75 | 1.0  |
| g./l.....                 | 0    | 0.6  | 0.9  | 1.2  |
| Final pH.....             | 2.9  | 2.4  | 2.5  | 2.5  |
| Chlorine dioxide, p.p.m.: |      |      |      |      |
| 0 minutes.....            | 0    | 0    | 0    | 0    |
| 15 minutes.....           | 400  | 75   | 90   | 90   |
| 30 minutes.....           | 380  | 115  | 115  | 115  |
| 60 minutes.....           | 310  | 140  | 130  | 130  |
| Brightness.....           | 85.1 | 88.3 | 87.5 | 87.1 |

The data show good pH control, material repression of chlorine dioxide formation even at this pH and excellent bleaching.

## Example XXII

Another aqueous concentrate suitable for use according to the present invention was made by dissolving the following components in the proportions indicated:

| Component                                          | Percent by weight |
|----------------------------------------------------|-------------------|
| Calcium nitrate.....                               | 20                |
| Ethylenediamine.....                               | 10                |
| Ethylenediamine tetra-acetic acid sodium salt..... | 5                 |
| Water.....                                         | 65                |
| Total.....                                         | 100               |

## Example XXIII

An aqueous concentrate was prepared by dissolving the following components in water in the proportions indicated:

| Component                                          | Percent by weight |
|----------------------------------------------------|-------------------|
| Sodium nitrate.....                                | 30                |
| Ethylenediamine.....                               | 10                |
| Ethylenediamine tetra-acetic acid sodium salt..... | 5                 |
| Water.....                                         | 55                |
| Total.....                                         | 100               |

A bleach bath was prepared by dissolving 1.0 gram per liter of 94 weight percent calcium chlorite in water. To separate 500 milliliter portions of this solution were added varying amounts of the concentrate described above, reserving one portion as a blank. Each portion was adjusted to pH 3.5 with 56 weight percent acetic acid, then heated to 85° C. for one hour. Nitrogen was bubbled through the solution during this time to sweep out the chlorine dioxide into a potassium iodide solution. At the end of one hour the total available chlorine and the chlorine dioxide remaining in the solution, the chlorine dioxide swept out, and the pH were determined. The following results were obtained:

| Test No.                                  | 1     | 2     | 3     |
|-------------------------------------------|-------|-------|-------|
| Concentrate added:                        |       |       |       |
| ml/l.....                                 | 0     | 0.50  | 1.50  |
| g/l.....                                  | 0     | 0.6   | 1.8   |
| Final pH.....                             | 4.1   | 3.6   | 3.55  |
| Available chlorine:                       |       |       |       |
| Initial, p.p.m.....                       | 1,535 | 1,535 | 1,535 |
| Final, p.p.m.....                         | 680   | 980   | 1,055 |
| Chlorine dioxide:                         |       |       |       |
| Swept out, p.p.m.....                     | 220   | 91    | 60    |
| In solution, p.p.m.....                   | 16    | 34    | 22    |
| Total chlorine dioxide formed, p.p.m..... | 236   | 125   | 82    |

The data show that the composition of this invention materially reduces chlorine dioxide evolution from calcium chlorite solution and maintains good pH control.

## Example XXIV

The following solid composition was prepared:

| Component                                          | Percent by weight |
|----------------------------------------------------|-------------------|
| Sodium nitrate.....                                | 40                |
| Disodium phosphate.....                            | 45                |
| Ethylenediaminedihydrochloride.....                | 10                |
| Ethylenediamine tetra-acetic acid sodium salt..... | 5                 |
| Total.....                                         | 100               |

Each component was finely ground and the mixture was homogenized by tumbling.

A bleach bath was prepared by dissolving one gram per liter of a commercial product containing 80 weight percent NaClO<sub>2</sub> and one gram per liter of the above composition in water. Formic acid was added to bring the pH to 2.5 and the solution was heated to 85° C. It was stirred and maintained at that temperature for one hour in contact with swatches of a polyethylene terephthalate fiber-cotton cloth (solution to cloth weight ratio, 30/1) and with a test piece of type 316 stainless steel. Chlorine dioxide content of the solution was determined from time to time and at the end of one hour the swatch was removed, rinsed, dried, ironed and the brightness determined using a Photovolt brightness meter with a "tristimulus" green filter (original brightness, 60.0). A blank was run omitting the solid repressor composition of the

present invention and the following comparative results were obtained:

|                           | Blank | With additive |
|---------------------------|-------|---------------|
| Chlorine dioxide, p.p.m.: |       |               |
| 0 minutes.....            | 0     | 0             |
| 15 minutes.....           | 125   | 100           |
| 30 minutes.....           | 150   | 130           |
| 60 minutes.....           | 160   | 150           |
| Brightness of cloth.....  | 80    | 81            |

The data show that chlorine dioxide was maintained at all times at a lower level in the bath with additive but the same bleaching effect was obtained in the same time.

## Example XXV

A bleach bath was prepared by dissolving one gram per liter of a commercial product containing 80 weight percent NaClO<sub>2</sub> and one gram per liter of the solid composition of Example XXIV in water. Acetic acid was added to bring the pH to 3.0 and the solution was heated to 85° C. It was stirred and maintained at that temperature for one hour in contact with a swatch of a polyethylene terephthalate fiber-cotton cloth (solution to cloth weight ratio, 30/1). Chlorine dioxide content of the solution was determined from time to time and at the end of one hour the swatch was removed, rinsed, dried, ironed and the brightness determined using a Photovolt brightness meter with a "tristimulus" green filter (original brightness, 60.0). A blank was run omitting the solid repressor composition of the present invention and the following comparative data were obtained:

|                           | Blank | With additive |
|---------------------------|-------|---------------|
| Chlorine dioxide, p.p.m.: |       |               |
| 0 minutes.....            | 0     | 0             |
| 15 minutes.....           | 95    | 18            |
| 30 minutes.....           | 120   | 45            |
| 60 minutes.....           | 165   | 80            |
| Brightness of Cloth.....  | 80    | 80            |

The data show very substantial repression of chlorine dioxide formation without any interference with the effectiveness of the bath in bleaching.

## Example XXVI

A bleach bath was prepared by dissolving one gram per liter of a commercial product containing 80 weight percent NaClO<sub>2</sub>, ferric chloride to provide 3 parts per million by weight of dissolved iron per liter and one gram per liter of the solid composition of Example XXIV. Acetic acid was added to bring the pH to 3. A swatch of a polyacrylonitrile fiber cloth was added (solution to cloth weight ratio, 30/1) and the mixture was stirred at 85° C. for one hour with a type 316 stainless steel stirrer. The cloth had an original brightness of 83 measured using a Photovolt brightness meter with a "tristimulus" green filter. Chlorine dioxide content of the solution was determined on samples removed at intervals. At the end of one hour, the cloths were removed, rinsed, dried, ironed and the brightness determined as before. A blank was run omitting the solid repressor composition of the present invention. The following results were obtained:

|                                     | Blank | Test |
|-------------------------------------|-------|------|
| Repressor composition added, g..... | 0     | 1    |
| Final pH.....                       | 4.2   | 3.0  |
| Chlorine dioxide content, p.p.m.:   |       |      |
| 0 minutes.....                      | 0     | 0    |
| 15 minutes.....                     | 100   | 20   |
| 30 minutes.....                     | 100   | 50   |
| 60 minutes.....                     | 90    | 100  |
| Brightness.....                     | 84.1  | 86.8 |

These data show maintenance of constant pH and low

17

chlorine dioxide formation. The bleach was improved over the blank without the represser composition.

*Example XXVII*

A bleach bath was prepared by dissolving one gram per liter of a commercial product containing 80 weight percent  $\text{NaClO}_2$ , ferric chloride to provide 3 parts per million by weight of dissolved iron per liter and one gram per liter of the solid composition of Example XXIV. A mixture of two volumes of concentrated nitric acid and one volume of glacial acetic acid was added to bring the pH of the solution to 2.5. Swatches of polyacrylonitrile fiber-cloth were added (solution to cloth ratio, 30/1) and the mixture was stirred at 85° C. for one hour. The cloth had an original brightness of 83 measured using a Photovolt brightness meter with a "tristimulus" green filter. Chlorine dioxide content of the solution was determined on samples removed at intervals. At the end of one hour, the cloths were removed, rinsed, dried, ironed and the brightness determined as before. A blank was run omitting the solid represser composition of the present invention. The following results were obtained:

|                                   | Blank | Test |
|-----------------------------------|-------|------|
| Represser composition added, g.   | 0     | 1    |
| Final pH                          | 2.9   | 2.4  |
| Chlorine dioxide content, p.p.m.: |       |      |
| 0 minutes                         | 0     | 0    |
| 15 minutes                        | 400   | 110  |
| 30 minutes                        | 380   | 150  |
| 60 minutes                        | 310   | 170  |
| Brightness                        | 85.1  | 87.8 |

These data show maintenance of constant pH and low chlorine dioxide formation. The bleach was improved over the blank without the represser composition.

*Example XXVIII*

The following solid composition was prepared by mixing the finely ground components:

| Component                                     | Percent by Weight |
|-----------------------------------------------|-------------------|
| Sodium nitrate                                | 51                |
| Disodium phosphate                            | 34                |
| Ethylenediamine dihydrochloride               | 10                |
| Ethylenediamine tetra-acetic acid sodium salt | 5                 |
| Total                                         | 100               |

A bleach solution was prepared by dissolving in water at 60° C., 17.2 grams of the above composition and 17.2 grams of a commercial product containing 80 weight percent  $\text{NaClO}_2$  to make each liter of solution. The solution was acidified to pH 3.8 by the addition of acetic acid. To one portion of the solution was added several swatches of cotton cloth using a solution to cloth weight ratio of 9:1. Another portion was tested without cloth. A third solution contained 17.2 grams per liter of a commercial product containing 80 weight percent  $\text{NaClO}_2$  acidified with acetic acid to pH 3.8, but containing no represser composition or cloth. All three solutions were maintained at 60° C. for 45 minutes. A stream of nitrogen was passed over each solution at 200 milliliters per minute. The chlorine dioxide was absorbed from the gas stream in acidified potassium iodide solution and the liberated iodine was titrated at the end of 45 minutes using standard sodium thiosulfate solution. The sweep-gas from the solution without represser contained 25 parts per million of chlorine dioxide, while the sweep-gas from the solutions containing the represser composition contained only 5.1 and 4.1 parts per million of chlorine dioxide from the solutions with and without cloth, respectively.

*Example XXIX*

A composition was prepared by mixing 6 grams of

75

18

ethylene diamine with 30 grams of sodium dihydrogen phosphate monohydrate. The mixture was moistened with one milliliter of water and stirring was continued while the mixture heated to 98° C. On cooling, the composition was ground and further mixed with 19 grams of disodium phosphate and 5 grams of ethylene diamine tetra-acetic acid sodium salt. The mixture was reground and then combined with 40 grams of sodium nitrate, ground again. The resulting powder was stable, odorless and suitable for use in acid chlorite solutions.

*Example XXX*

A mixture was prepared by stirring 6 grams of triethylene tetra-amine with 30 grams of sodium dihydrogen phosphate monohydrate. On the addition of one milliliter of water and stirring, the mixture heated to about 80° C. It was maintained in an oven at 90° C. for one hour, cooled and ground. This composition was mixed with 19 grams of disodium phosphate, 5 grams of ethylene diamine tetracetic acid sodium salt and 40 grams of sodium nitrate, all of which were ground together to provide another solid composition of the present invention.

*Example XXXI*

A bleach bath was prepared by dissolving one gram per liter of 94 percent calcium chlorite and one gram per liter of the solid composition of Example XXIV in water. Acetic acid was added to bring the pH to 3.5. The solution was heated to 85° C. and stirred for one hour. A stream of nitrogen sweeping over the surface at 200 cc./min. swept all chlorine dioxide released into a trap containing aqueous potassium iodide. At the end of one hour the chlorine dioxide dissolved in the solution, the chlorine dioxide swept off, and the total available chlorine in the solution were determined. A blank was run omitting the composition of this invention and the following comparative data were obtained:

|                                    | Blank | With Additive |
|------------------------------------|-------|---------------|
| Available chlorine:                |       |               |
| Initial, p.p.m.                    | 1,535 | 1,525         |
| Final, p.p.m.                      | 775   | 1,035         |
| $\text{ClO}_2$ swept out, p.p.m.   | 145   | 47            |
| $\text{ClO}_2$ in solution, p.p.m. | 34    | 71            |
| Total $\text{ClO}_2$ evolved       | 179   | 118           |

The data show that the composition of this invention substantially reduces chlorine dioxide formation from solutions of calcium chlorite. This example shows the effectiveness of the represser with respect to calcium chlorite.

What is claimed is:

1. An aqueous acidic bleaching bath having an acid pH within the range of from 2 to 7 and consisting essentially of water, a water-soluble metal chlorite selected from the group consisting of alkali metal chlorites and alkaline earth metal chlorites, and at least one polyamine of the formula
  2. The aqueous acidic bleaching bath of claim 1 wherein the water-soluble metal chlorite is an alkali metal chlorite.
  3. The aqueous acidic bleaching bath of claim 1 wherein the water-soluble metal chlorite is sodium chlorite.
  4. The aqueous acidic bleaching bath of claim 1 wherein the polyamine is ethylene diamine.
  5. The aqueous acidic bleaching bath of claim 1
- $\text{NH}_2(\text{CH}_2\text{CHR}\cdot\text{NH})_n\text{H}$
- in an amount sufficient to prevent the evolution of chlorine dioxide gas from the bath but insufficient in amount to destroy the bleaching power of the chlorite, R being selected from the group consisting of hydrogen and methyl and n being an integer from 1 to 4.

wherein the water-soluble metal chlorite is an alkali metal chlorite and the polyamine is ethylene diamine.

6. The aqueous acidic bleaching bath of claim 1 wherein the water-soluble metal chlorite is sodium chlorite and the polyamine is ethylene diamine.

7. The aqueous acidic bleaching bath of claim 1 wherein the polyamine is propylene diamine.

8. The aqueous acidic bleaching bath of claim 1 wherein the polyamine is triethylene tetramine.

9. The aqueous acidic bleaching bath of claim 1 wherein the polyamine is dipropylene triamine.

10. The aqueous acidic bleaching bath of claim 1 in which the pH range is from 2 to 4.

11. The aqueous acidic bleaching bath of claim 1 in which the polyamine is present in the proportion of 10 to 1,000 parts per million by weight per 1,000 to 2,000 parts per million by weight of sodium chlorite.

12. An aqueous concentrate suitable for use in an aqueous acidic chlorite bleaching bath having an acid pH within the range of from 2 to 7, said chlorite being a water-soluble metal chlorite selected from the group consisting of alkali metal chlorites and alkaline earth metal chlorites, said concentrate consisting essentially of 20 to 32 weight percent of at least one compound selected from the group consisting of alkali metal nitrates and alkaline earth metal nitrates, 5 to 15 weight percent of at least one polyamine of the formula



R being selected from the group consisting of hydrogen and methyl and n being an integer from 1 to 4, 3 to 10 weight percent of a chelating agent for deleterious metal ions and which is stable with respect to the metal chlorite and effective in the acid bath, and a balance of water.

13. The aqueous concentrate of claim 12 wherein the compound selected from the group consisting of alkali metal nitrates and alkaline earth metal nitrates is sodium nitrate.

14. The aqueous concentrate of claim 12 wherein the polyamine is ethylene diamine.

15. The aqueous concentrate of claim 12 wherein the chelating agent is ethylene diamine tetra-acetic acid.

16. The aqueous concentrate of claim 12 wherein the compound selected from the group of alkali metal nitrates and alkaline earth metal nitrates is sodium nitrate, the polyamine is ethylene diamine and the chelating agent is ethylene diamine tetra-acetic acid.

17. A solid composition suitable for use in an aqueous acidic chlorite bleaching bath having an acid pH within the range of from 2 to 7, said chlorite being a water-soluble metal chlorite selected from the group consisting of alkali metal chlorites and alkaline earth metal chlorites, said composition consisting essentially of 30 to 55 weight percent of at least one alkali metal nitrate, 25 to 50 weight percent of a buffering agent, 4 to 12 weight percent of at least one polyamine of the formula



R being selected from the group consisting of hydrogen and methyl and n being an integer from 1 to 4, and 3

to 20 weight percent of a chelating agent for deleterious metal ions and which is stable to the metal chlorite and effective in the acid bath.

18. The solid composition of claim 17 wherein the alkali metal nitrate is sodium nitrate.

19. The solid composition of claim 17 wherein the buffering agent is disodium phosphate.

20. The solid composition of claim 17 wherein the polyamine is ethylene diamine hydrochloride.

21. The solid composition of claim 17 wherein the chelating agent is ethylene diamine tetra-acetic acid.

22. The solid composition of claim 17 wherein the alkali metal nitrate is sodium nitrate, the buffering agent is disodium phosphate, the polyamine is ethylene diamine, and the chelating agent is ethylene diamine tetra-acetic acid.

23. In the use of an aqueous acidic chlorite bleaching bath having an acid pH within the range of from 2 to 7, said chlorite being a water-soluble metal chlorite selected from the group consisting of alkali metal chlorites and alkaline earth metal chlorites, the method of repressing the generation of chlorine dioxide in the bath which comprises including in the bath at least one polyamine of the formula



in an amount sufficient to prevent the evolution of chlorine dioxide gas from the bath but insufficient in amount to destroy the bleaching power of the chlorite, R being selected from the group consisting of hydrogen and methyl and n being an integer from 1 to 4.

24. The method of claim 23 in which the bath has a pH range of from 2 to 4.

25. The method of claim 23 in which the polyamine is included in the bath in the proportion of 10 to 1,000 parts per million by weight per 1,000 to 2,000 parts per million by weight of sodium chlorite.

#### References Cited in the file of this patent

#### UNITED STATES PATENTS

|           |               |               |
|-----------|---------------|---------------|
| 1,748,494 | Murrill       | Feb. 25, 1930 |
| 2,377,066 | Baird et al.  | May 29, 1945  |
| 2,499,987 | Clapham       | Mar. 7, 1950  |
| 2,526,839 | Ashton        | Oct. 24, 1950 |
| 2,711,363 | Waibel        | June 21, 1955 |
| 2,739,882 | Ellis         | Mar. 27, 1956 |
| 2,740,689 | Easton et al. | Apr. 3, 1956  |
| 2,810,717 | Lamborn       | Oct. 22, 1957 |
| 2,836,566 | Duncan        | May 27, 1958  |
| 2,850,461 | Bloch et al.  | Sept. 2, 1958 |

#### FOREIGN PATENTS

|         |        |              |
|---------|--------|--------------|
| 507,997 | Canada | Dec. 7, 1954 |
|---------|--------|--------------|

#### OTHER REFERENCES

Versenes: Tech. Bull. No. 2, sec. II, pp. 6-10, 16, 17, pub. by Bersworth Chemical Co., Framingham, Mass. (1952).